

# UNITED STATES PATENT OFFICE.

EARL V. WAGNER, OF SCRANTON, PENNSYLVANIA, ASSIGNOR TO WAGNER FIRE BRICK COMPANY, OF HELENA, MONTANA.

## PLASTIC COMPOSITION FOR MAKING FIRE-BRICKS.

1,209,784.

Specification of Letters Patent. Patented Dec. 26, 1916

No Drawing. Original application filed January 8, 1916, Serial No. 70,983. Divided and this application filed August 5, 1916. Serial No. 113,221.

To all whom it may concern:

Be it known that I, EARL V. WAGNER, a citizen of the United States, residing at Scranton, in the county of Lackawanna and 5 State of Pennsylvania, have invented a new and useful Plastic Composition for Making Fire-Bricks, of which the following is a specification.

My composition consists of the following 10 named ingredients combined in substantially the proportions here stated, namely: coal ash, 100 pounds; alumina, 2 pounds; water, 2 to 2½ gallons.

It is not intended to confine the discovery 15 here applied for to the use of the ingredients specified in the proportions stated, as these proportions may in some cases be advantageously varied producing substantial identity of result. To illustrate: If the fusion 20 point of the coal ash is found to be less than 2600 degrees Fahrenheit, or if a high fusion point for the fire bricks is desired, the percentage of alumina used is to be increased. Thus, taking 100 pounds of coal ash as a 25 basis whose fusion point is 2600 degrees Fahrenheit, to this is added 2 pounds of alumina which will raise the fusion point of the mixture to 3000 (2950 to 3100) degrees 30 Fahrenheit. If on account of foreign substances in the coal ash its fusion point is found to be below 2600 degrees Fahrenheit the percentage of alumina must be correspondingly increased to produce the above named result, the percentages being based 35 upon the original fusion point of the coal ash and upon the fusion point of the fire bricks which it is desired to obtain. The proportions above stated are therefore for approximately pure coal ash having a fusion 40 point of approximately 2600 degrees Fahrenheit.

Grind and mingle the coal ash with the alumina, then add the water and mix until thoroughly plastic. Press the plastic mass 45 through a molding machine of approved type. Cut the bricks to the size desired by the use of a cutting machine of approved type. The freshly cut bricks are then re-

pressed in a repressing machine of approved type in which they are subjected to heavy 50 pressure sufficient to fill out all angles and decrease the laminations and to strengthen the bond. Then place the bricks in a closed drying oven and dry for six to eight hours at a temperature of 500 to 600 degrees 55 Fahrenheit. Remove the bricks while hot to a closed burning kiln whose temperature is gradually increased from 2200 to 2400 degrees Fahrenheit at which temperature the bricks are fired for seven to eight days, 60 when they are allowed to cool gradually, resulting in the finished product.

I am aware that prior to my invention and discovery various quantities of coal ashes have been mixed with clay for the purpose of producing vitrified paving bricks having practically no porosity and consequently no absorptive qualities. I am also aware that it has been attempted to manufacture fire bricks from mixtures of coal 70 ashes, shale and fire clay; that fire bricks may be produced without the addition of coal ashes from mixtures of clay and difficultly fusible materials, such as ground burnt fire clay. I am not aware, however, that 75 fire bricks having the necessary porous and heat resisting qualities and adequate crushing strength to make them commercially valuable have ever been produced from a mixture consisting essentially of finely 80 ground coal ashes with the addition of only a small proportion of alumina such as specified above, or that the ingredients specified have been mixed, molded and burned in any other proportions to make fire bricks, prior 85 to my invention and discovery thereof.

What I claim:

The herein described plastic composition for making fire bricks, consisting of coal ashes, one hundred pounds; alumina two 90 pounds; water two to two and one-half gallons, substantially as described.

EARL V. WAGNER.

Witnesses:

I. B. POTTER,  
A. G. DAVIS.

Correction in Letters Patent No. 1,209,784.

It is hereby certified that the name of the assignee in Letters Patent No. 1,209,784, granted December 26, 1916, upon the application of Earl V. Wagner, of Scranton, Pennsylvania, for an improvement in "Plastic Composition for Making Fire-Bricks," was erroneously written and printed "Wagner Fire Brick Company," whereas the name of the assignee should appear as *The Wagner Fire Brick Company*, as shown by the records of assignments in this office; and that the said Letters Patent should be read with this correction therein that the same may conform to the record of the case in the Patent Office.

Signed and sealed this 6th day of March, A. D., 1917.

[SEAL.]

F. W. H. CLAY,

*Acting Commissioner of Patents.*

Cl. 106—11.